

# United States Patent [19]

Dean et al.

[11] 3,887,731

[45] June 3, 1975

[54] **CORROSION RESISTANT COATING SYSTEM FOR FERROUS METAL ARTICLES HAVING BRAZED JOINTS**

[75] Inventors: **Michael F. Dean; Hossein Borougerdi; John A. Puchot**, all of San Antonio, Tex.

[73] Assignee: **Chromalloy American Corporation**, New York, N.Y.

[22] Filed: **Apr. 23, 1973**

[21] Appl. No.: **353,677**

[52] U.S. Cl. .... **427/258**; 29/195; 29/196.2; 148/6.16

[51] Int. Cl. .... **C23c 9/00**

[58] Field of Search .... 148/6.16; 117/71, 135.1, 117/127; 29/195 M, 196.2, 196.6

[56] **References Cited**

UNITED STATES PATENTS

|           |         |               |          |
|-----------|---------|---------------|----------|
| 3,047,420 | 7/1962  | Bernick ..... | 117/71 M |
| 3,338,733 | 8/1967  | Rowady .....  | 117/71 M |
| 3,498,823 | 3/1970  | Jones .....   | 117/71 M |
| 3,544,348 | 12/1970 | Boone .....   | 117/71 M |

|           |         |                   |          |
|-----------|---------|-------------------|----------|
| 3,721,534 | 3/1973  | Kubick .....      | 117/71 M |
| 3,723,162 | 3/1973  | Leontaritis ..... | 117/71 M |
| 3,764,371 | 10/1973 | Baldi .....       | 148/6.16 |

Primary Examiner—L. Dewayne Rutledge  
Assistant Examiner—Arthur J. Steiner  
Attorney, Agent, or Firm—Hopgood, Calimafde, Kalil

[57] **ABSTRACT**

Ferrous metal articles, such as stainless steel articles, characterized by at least one brazed joint, in which the braze is a non-ferrous alloy are aluminized by first selectively coating the braze alloy with nickel and then thermally diffusing aluminum over the entire surface of the article including the selectively coated braze, such that a sacrificial corrosion resistant coating is produced wherein the aluminum coating on the ferrous metal surface is characterized by the presence of iron aluminide, and wherein the aluminum coating on the nickel-coated braze is characterized by the presence of nickel aluminide. The aluminide coatings are further enhanced by the application of a non-metallic coating, e.g. a conversion coating.

**15 Claims, 3 Drawing Figures**



FIG. 1



FIG. 2



FIG. 3

# CORROSION RESISTANT COATING SYSTEM FOR FERROUS METAL ARTICLES HAVING BRAZED JOINTS

This invention relates to the protection of ferrous metal articles against corrosion in highly saline and/or marine or other corrosive environments by employing thermally diffused aluminum as the main sacrificial coating, the invention being particularly applicable to ferrous metal articles, such as stainless steel articles, characterized by at least one brazed joint, wherein the braze is a non-ferrous alloy. The invention also relates to the production of aluminized coatings on ferrous metal articles comprising brazed joints and also having a barrier-type non-metallic overcoat.

## FIELD OF THE INVENTION

Jet and gas turbine engine compressor components are subject to corrosion in highly saline environments at the air intake end of the engine and also to the direct impact of abrasive particulate matter, such as coral dust. Additionally, the compressor blades are subjected to tremendous mechanical stresses from centrifugal forces, thermal shock, vibration and other sources of stresses. Thus, corrosion can accelerate catastrophic failure, since pits and other corrosion defects can act as stress raisers.

High strength ferrous alloys are employed in the construction of compressor blades and other aircraft engine components such as vane/shrouds (e.g. Society of Automotive Engineers allow designation AMS 5508, AMS 5616, AMS 6304 and others) but, because of their low resistance to saline corrosion, they are generally provided with a protective surface treatment. One in particular is the provision of an aluminum-base diffusion coating on the ferrous substrate by pack-aluminizing at coating temperatures ranging up to 1,000 F and preferably not higher so as to avoid undesired crystallographic or metallurgical changes in the substrate during coating which might have an adverse or undesired effect on the mechanical property of the parts. Such coatings have provided advantageous oxidation and erosion resistance and have minimized the production of pulverous corrosion by-products and have been very useful in extending operating life of jet engine components.

However, where the jet and gas turbine engine components are comprised of at least one brazed joint, such as vane/shroud assemblies in which the braze is a non-ferrous alloy based on a metal selected from the group consisting of copper, silver and gold, e.g. copper-silver- and/or gold-base brazing alloys, certain problems arise in the production of a uniform aluminized coating having requisite physical characteristics. The braze, being markedly different than the ferrous metal surface, reacts differently during the diffusion of aluminum therein. The extent of diffusion of aluminum in different materials is governed mainly by the aluminide phases that are formed which act as diffusion barriers. Generally speaking, the lower the melting point of a particular braze alloy, the deeper is the diffusion of aluminum into it.

Thus, in the case of aluminum diffusion in a brazed component in which stainless steel elements are brazed together to form the joints, the aluminum case depth on the stainless steel element might be 0.0005 inch, whereas the aluminum may penetrate as much as 0.007

inch deep into the brazed portions of the joints for a braze alloy comprising by weight 50% Ag, 18% Cd, 16% Zn and 16% Cu; or as much as 0.002 inch for a braze composition comprising by weight 54% Ag, 40% Cu and 6% Zn.

Mechanical tests have indicated that the uncontrolled diffusion of aluminum into the braze alloy tends to degrade the brazed joint as evidenced by fatigue test data.

Thus, it would be desirable to provide a method of controlling the diffusion at the brazed joint commensurate with the diffusion at the unbrazed portion of the component such as to insure uniform properties over the whole surface of the component.

## OBJECTS OF THE INVENTION

It is thus the object of the invention to provide a sacrificial coating of aluminum on ferrous metal parts characterized by the presence of at least one brazed comprising a non-ferrous brazing alloy and wherein the properties of the coating are substantially uniform at both the unbrazed areas and the brazed joint.

Another object of the invention is to provide a method of aluminizing a ferrous metal part having at least one brazed joint, wherein the braze at the joint is selectively coated with a layer of nickel prior to aluminizing of the whole part such that the fatigue properties at the joint are maintained at acceptable levels or are enhanced.

A further object is to provide, as an article of manufacture, an aluminized ferrous metal part, such as a stainless steel aircraft part, characterized by at least one brazed joint of non-ferrous metal or alloy, the braze having been first provided with a layer of nickel, such that the aluminum coating in the unbrazed area at the steel substrate is characterized by the presence of iron aluminide and in the brazed areas by the presence of nickel aluminide.

A still further object is to provide a method of preparing a ferrous metal part having at least one brazed joint for aluminizing wherein the brazed joint is selectively plated with a coating of nickel while inhibiting nickel from plating out in the unbrazed areas.

These and other objects will more clearly appear from the following disclosure and the accompanying drawings.

## DRAWINGS

FIG. 1 represents a vane/shroud assembly of stainless steel in which the vanes are brazed across the annular space between inner and outer rings making up the shroud;

FIG. 2 is a close-up of a fragment of the shroud showing the plurality of brazed joints making up the vane-/shroud assembly; and

FIG. 3 is a representation of a micrograph of a brazed joint at 100 times magnification.

## STATEMENT OF THE INVENTION

One aspect of the invention resides in a method of aluminizing a brazed ferrous metal article, such as an aircraft engine component comprised of at least one brazed joint. The brazing material in the joint is made of a nonferrous brazing alloy having a melting point ranging from about 1125°F (607°C) to 1925°F (1052°C), such as an alloy based on at least one metal selected from the group consisting of copper, silver and

gold. Because the aluminum tends to diffuse more deeply into the non-ferrous brazing alloy than in the steel substrate, the method resides in selectively coating the brazed area with nickel and then thermally diffusing the aluminum, preferably by pack cementation, into the entire surface of the ferrous component, including the selectively coated brazed area and thereby produce a substantially uniform coating of aluminum, wherein the thermally diffused aluminum coating on the ferrous metal surface outside the brazed area is characterized by the presence of iron aluminide and wherein the thermally diffused aluminum coating on the nickel coated braze is characterized by the presence of nickel aluminide. Fatigue tests on cantilevered specimens have indicated that the fatigue properties of the aluminized nickel-coated brazed specimens are comparable to uncoated specimens and superior to aluminized brazed specimens without the nickel protective layer.

The foregoing method is also applicable to the coating of ferrous metal articles which uses a protective duplex coating system, that is, a system in which following the production of a thermally aluminized coating on the ferrous metal substrate, a non-metallic silicate overcoat is applied to the aluminum coating which is

and preferably 1175°F (635°C) to 1850°F (1010°C). As will be understood by those skilled in the art, the non-ferrous brazing alloy must have a lower melting point than the metal substrates being joined and yet must be high enough to resist softening at elevated temperatures to which the aircraft part (e.g. vane/shroud assemblies) is subjected during use.

Examples of non-ferrous brazing alloy compositions commonly employed for producing brazed joints in aircraft components made of ferrous metals, e.g. stainless steel are by weight as follows: (1) 50% Ag, 18% Cd, 16% Zn and 16% Cu [designated as AMS 4770 C]; (2) 54% Ag, 40% Cu, 6% Zn and up to 1% Ni [designated as AMS 4772 B]; (3) 82% Au, 18% Ni [designated as PWA 698]; (4) 54% Ag, 25% Pd and 21% Cu [designated as PWA 706] and (5) 55% Cu, 35% Mn and 10% Ni among many others. The diffusion of aluminum in alloy (1) may proceed up to a depth of 0.007 inch and in the others up to 0.002 inch. Such diffusion by aluminum into the braze has a weakening effect on the joint and adversely affects its resistance to fatigue.

Illustrative brazing alloy compositions range in weight percent (for brazing stainless steel) including their solidus, liquidus and brazing temperatures are as follows:

| Exam-<br>ple<br>Nos. | % Ag  | % Cu      | % Zn      | % Cd  | % Ni    | Solidus | Liquidus | Temperature °F<br>Brazing |
|----------------------|-------|-----------|-----------|-------|---------|---------|----------|---------------------------|
| 1A                   | 44-46 | 14-16     | 14-18     | 23-25 | —       | 1125    | 1145     | 1145-<br>1400             |
| 2A                   | 49-51 | 14.5-16.5 | 14.5-18.5 | 17-19 | —       | 1160    | 1175     | 1175-<br>1400             |
| 3A                   | 49-51 | 14.5-16.5 | 13.5-17.5 | 15-17 | 2.5-3.5 | 1170    | 1270     | 1270-<br>1500             |
| 4A                   | 39-41 | 29-31     | 26-30     | —     | 1.5-2.5 | 1240    | 1435     | 1435-<br>1650             |
| 5A                   | 44-46 | 29-31     | 23-27     | —     | —       | 1250    | 1370     | 1370-<br>1550             |
| 6A                   | 54    | bal.      | 5         | —     | 1       | 1325    | 1575     | 1575-<br>1785             |
| 7A                   | 60    | bal.      | —         | —     | 10% Sn  | 1115    | 1325     | 1325-<br>1550             |
| 8A                   | 92.5  | bal.      | —         | —     | 0.2 Li  | 1435    | 1635     | 1610-<br>1800             |

highly adherent. With respect to the non-metallic overcoat, reference is made to co-pending application Ser. No. 143,842, filed May 17, 1971. The disclosure of said application relating to the production of such non-metallic non-metallic on aluminized ferrous metal surfaces is incorporated herein by reference.

As stated hereinbefore, the non-ferrous brazing alloys which present the problem of uncontrolled diffusion of aluminum therein preferably include those which are based on one or more metals selected from the group consisting of copper, silver and gold. When the expression "based on one or more metals of the group copper, silver and gold" is employed, what is meant is that the non-ferrous brazing alloy contains at least one of the foregoing copper group metals as a main ingredient, with one or more of other non-ferrous metals making up substantially the balance, such as zinc, nickel, palladium, cadmium, tin, manganese, and the like.

Apparently, the lower the melting point of the braze alloy, the deeper is the aluminum diffusion into it. Thus, it may be stated generally that the non-ferrous brazing alloys include those having melting points ranging from about 1125°F (607°C) to 1925°F (1052°C)

45 Another brazing alloy based on gold comprises 81.5% Au and the balance nickel. This alloy has a solidus-liquidus temperature of 1740°F and is employed over a brazing temperature of about 1740°F to 1840°F.

50 Most stainless steels can be brazed by any one of several different filler metals, including silverbase alloys, gold-base alloys, copper-base alloys and the like. Stating it another way, the non-ferrous brazing alloy may contain at least about 40 percent by weight of the copper group metals and preferably at least about 50% and the balance non-ferrous alloying ingredients so long as the melting point of the alloy ranges from about 1125°F to 1925°F and preferably from about 1175°F to 1850°F. The melting point is generally taken as the liquidus temperature of the alloy. The minimum of at least 55 40 percent of the copper group metal is met where the alloy contains at least 40% Ag, or 40% cu or 40% Au, or at least 40% of a combination of two or more of the foregoing copper group metals. As stated hereinbefore, the other non-ferrous alloying elements may comprise one or more of Zn, Cd, Ni, Sn, Mn, Pd and the like. Thus, the brazing alloy may contain 40 to 95% of at least one of the copper group metals and the balance at least one other non-ferrous metal.

When the foregoing brazing alloys are employed in the production of certain aircraft components, it has been found essential to selectively coat the brazed areas with nickel before thermally aluminizing the whole component. Various methods may be employed in selectively coating the brazed joint with nickel. One method is to apply a resist to the unbrazed areas (e.g. a thin wax coating) while leaving the brazed portion of the joint exposed for nickel plating. Following nickel plating of the braze, the resist is removed from the component and the component then embedded in an aluminizing pack containing alumina, some aluminum powder and a small but effective amount of a halide e.g.  $\text{AlCl}_3$ . The use of the foregoing halide is advantageous in that very good aluminum coating can be produced at temperatures ranging up to about 1000°F (538°C) while avoiding the production of undesired crystallographic or metallurgical changes in the substrate. The aluminizing temperature should not exceed the melting point of the braze, otherwise, the brazed joint will be deleteriously affected during aluminizing.

The aluminized surface produced in the foregoing manner is characterized metallographically by the presence of iron aluminide in the unbrazed areas adjacent the ferrous substrate outside of the brazed portions and by the presence of nickel aluminide at the nickel-plated braze portions.

Where the aircraft component is made of stainless steel, such as those bearing the designations AMS 5508, AMS 5616, AMS 6304, 17-4PH, type 410 and others, we prefer to produce the nickel mask on the brazed areas by chemical plating. We find this method to be very advantageous in that we can passivate the exposed stainless steel substrate while activating the brazed areas, such that during the subsequent step of chemical plating, the nickel selectively coats only the brazed areas and not the stainless steel substrate.

Of the foregoing steels, the composition of AMS 5616 comprises 13% Cr, 2% Ni, 3% W and the balance essentially iron; type 410 comprises about 11.5 to 13.5% Cr, 1% Si max., 1 percent Mn max., 0.15% C max., and the balance essentially iron; and 17-4 PH comprises about 17% Cr, 4% Ni, 3% Cu, small amounts of Co, Mn, Si, etc., and the balance essentially iron. Broadly speaking, the steels may comprise about 5% to 25% Cr, up to 5% W, up to 25% Ni, up to 4% Cu, up to 3% Al, up to 2% Ti and the balance essentially iron.

The passivation of the steel substrate is achieved by employing a chemical anodizing solution comprised of cupric chloride, mercuric chloride, bismuth chloride, hydrochloric acid, alcohol and water. Broadly, the aqueous solution may have the following composition calculated in grams per liter (gpl) and milliliters per liter (ml/l):

10 to 70 gpl cupric chloride  
20 to 140 gpl mercuric bichloride  
10 to 70 gpl bismuth chloride  
100 to 400 ml/l of ethyl alcohol and  
100 to 400 ml/l concentrated hydrochloric acid  
balance essentially water to make one liter equivalent.

Examples of actual bath compositions are as follows:

|                           | I    | II   | III  | IV   |
|---------------------------|------|------|------|------|
| Cupric chloride (gpl)     | 60   | 30   | 20   | 12   |
| Mercuric Bichloride (gpl) | 120  | 60   | 40   | 28   |
| Bismuth Chloride (gpl)    | 60   | 30   | 20   | 12   |
| Ethyl Alcohol (ml/l)      | 300  | 150  | 100  | 60   |
| Hydrochloric Acid (ml/l)  | 375  | 188  | 125  | 75   |
| Water (ml/l)              | bal. | bal. | bal. | bal. |

10 The foregoing solutions are used at room temperature, the steel parts being immersed therein for generally about  $\frac{1}{4}$  to 10 minutes.

Following preparation of the solution, the cleaned stainless steel component (e.g. in the gritblasted honed condition) is immersed in it. The steel surface tends to darken while mercury reduction occurs cathodically (due to galvanic action) on the braze at immersion times of  $\frac{1}{4}$  to 10 minutes. However, chemical or electroless plating of nickel will not occur on the surfaces of the component unless the steel substrate is further treated. This is done by subsequent nitric or chromic acid dipping at room temperature to remove any observable mercury, thereby activating the braze surface.

25 Typical passivating solutions for this treatment are: (a) 50 percent nitric acid solution, (B) saturated chromic acid solution, and (C) or varying combinations of both.

Following nitric acid dipping, the stainless steel component is then nickel plated in a chemical or electroless plating bath of nickel, such as nickel baths based on dimethylamine borane or sodium hypophosphite. The aqueous sodium hypophosphite may comprise the following:

|                      |              |
|----------------------|--------------|
| Nickel sulfate       | 15 to 30 gpl |
| Sodium Hypophosphite | 15 to 30 gpl |
| Sodium Glycolate     | 20 to 40 gpl |
| Sodium Succinate     | 10 to 20 gpl |

30 40 The pH is adjusted to 4.5 to 6.

The temperature is preferably 180°-195°F.

A typical aqueous solution is one containing 25 gpl nickel sulfate, 25 gpl sodium hypophosphite, 30 gpl sodium glycolate 17 gpl sodium succinate.

45 50 Chromium-containing steel components have been immersed for one hour to deposit approximately 0.0005 inch of nickel and for as long as 2 hours to produce a nickel plate approaching 0.001 inch thick on the braze, while inhibiting nickel plating out on the stainless steel substrate. Nickel plates found adequate for the purpose generally exceed about 0.0002 inch.

A stainless part that has been successfully treated in the foregoing manner is the vane/shroud component shown in FIGS. 1 to 3. FIG. 1 shows a vane/shroud 10 of AMS 5616 steel comprising inner and outer rings 11 and 12, respectively, with vanes 13 brazed therebetween.

55 60 The brazed joints 14 are clearly shown in FIG. 2. Referring to FIG. 3, vane 13 is shown attached by braze 14 to inner ring 11. The fillet of the AMS 4772B brazed joint has been selectively coated with nickel such that following aluminizing of the part by pack cementation, a layer 15 containing nickel aluminide is provided following the contour of the fillet. As will be noted, an aluminide layer 16 is shown adjacent the surface of the inner ring comprising iron aluminide by reaction with the steel substrate during pack cementation. As will

also be noted in FIG. 3, the specimen has an overplate of copper and nickel 17 to provide the necessary support for mounting and polishing said specimen without adversely affecting the coating.

In thermally aluminizing the selectively nickel-plated vane/shroud component shown in FIG. 1, a preferred pack cementation method is employed as follows:

The method comprises preparing an aluminizing pack comprised for example, of 800 lbs. of -60+140 mesh aluminum powder blended with 200 lbs. of  $\text{Al}_2\text{O}_3$ , also -60+140 mesh size. To the 1000 lb. mixture is added 30 lbs. of dry  $\text{AlCl}_3$  under a humidity preferably not exceeding 45 percent.

The pack is mixed in a vibrating blender under dry conditions for about 5 to 10 minutes. If the charge is a fresh charge, it is subjected to burn-out at 795°-825°F (425°C to 440°C) for 35 hours. However, where a charge has already been used and is recycled for another pack, burn-out is not required. The pack is placed in a dry condition in a retort with the vane-/shroud component of AMS 5616 steel to be treated, the vane/shroud being completely embedded in the pack using vibration to fill in the spaces between the vanes. The cover is sealed to the retort body with multiple layers of aluminum foil in the form of a gasket sufficient to prevent air from getting in but to allow outgassing of gaseous by-products.

The retort is placed in an oven ambient ambient temperature and the temperature allowed to rise to the desired coating temperature by the application of heat. As the temperature rises, it is preferred that it go through an endothermic arrest at about 350°F (176°C) due to vaporization of  $\text{AlCl}_3$  to effect further cleansing of the surface of the component of any oxide film thereon and then allowed to reach a temperature not exceeding about 1000°F (538°C), for example, a range of about 795°F to 825°F (425°C to 440°C) and the retort maintained at substantially that temperature range for about 36 hours. Upon completion of the heating cycle, the retort is removed from the oven and allowed to cool approximately to 400°F (205°C), after which it is placed in a dry environment for cooling to ambient temperature.

The cooled retort is then placed in a humidity control cabinet, the cover removed and the aluminum-coated vane/shroud taken out of the cementation pack. The part is cleaned of adhering coating compound by blowing with dry air and immersed in water to remove fine dust and other residues to provide a very clean aluminum deposit containing an iron aluminide intermetallic compound, such as  $\text{FeAl}_3$ , on the braze-free portion of the component and a nickel aluminide intermetallic compound on the nickel-plated brazed portion of the component. The aluminized surface, like other thermally diffused aluminum coatings, is characterized by sacrificial properties in that it will corrode in preference to the ferrous substrate in saline environments and, therefore, substantially protect the ferrous substrate against corrosion.

Generally speaking, the pack composition may comprise by weight about 60 to 100 percent aluminum, about 1 to 5 percent dry  $\text{AlCl}_3$  and the balance essentially a stable inert refractory oxide.

As stated hereinbefore, unless the braze of the joint is nickel plated prior to aluminizing the stainless steel component, the fatigue properties at the joint are generally degraded. This has been confirmed by tests in

which specimens of the joint have been subjected to cantilever loading to provide maximum bending stress at the joint during fatigue testing. In a test series conducted, the fatigue samples were shaped in the form of a "tee" from type 410 stainless steel by brazing a machined cantilever arm to the surface of the sample with alloy AMS 4772B. Prior to brazing, the specimens were solution treated, quenched and tempered.

In one specimen, the brazed joint was aluminized in the manner described hereinbefore without applying a nickel plate. That is to say, the braze was bare prior to aluminizing. In another specimen, the braze was first selectively nickel plated and subsequently aluminized. The aluminized specimens are then subjected to an oxidation/corrosion/fatigue screening test using the following cycle:

1. 10,000 fatigue cycles at 50,000 psi root load
2. 5 hours oxidation at 700°F
3. 16 hours salt spray

The salt spray test used is ASTM B117.

The foregoing cycle is repeated until the sample fails. The results on the bare brazed joint and the aluminized nickel-plated brazed joint are as follows:

| Specimen            | Total Number of Cycles | Fatigue Cycles to Failure at 50,000 psi | Salt Spray Hours | Oxidation Hours |
|---------------------|------------------------|-----------------------------------------|------------------|-----------------|
| Bare Joint          | 5                      | 58,000                                  | 80               | 25              |
| Nickel-Plated Joint | 19                     | 200,000*                                | 304              | 95              |

\*This specimen did not fail.

The failed joint showed general oxidation and corrosion attack to a depth of 0.0035 inch. The nickel-plated joint showed no evidence of braze corrosion after 19 test cycles. A bare joint without corrosion ran 300,000 cycles to failure at a load of 50,000 psi.

One of the attributes of an aluminide coating on a metal substrate is its ability to absorb readily a silicate liquid in the production of a protective nonmetallic overcoat.

As pointed out in the aforementioned copending application Ser. No. 143,842, it is believed that the high affinity of the thermally aluminized coating or surface for the silicate is associated with the physical-chemical character of the aluminized surface arising out of the method of growth of the aluminide. The expression "thermally aluminized coating or surface" is meant to cover the thermal diffusion of aluminum in a metal surface in which iron and/or nickel aluminide is formed at the surface.

In one embodiment, the non-metallic overcoat or barrier layer is formed by applying to the thermally aluminized surface of the article a solution of a soluble silicate salt at a temperature ranging up to about 100°C, for example, about 70°C to 95°C (about 160°F to 200°F), removing excess liquid from the surface, such as by blowing it off with air, to form a uniform layer of said silicate salt, and then drying the layer on said surface.

While the aluminized surface in and of itself exhibits resistance to saline corrosion, a typical salt spray test shows that sacrificial products form on the aluminized surface after approximately 15 hours of testing, whereas times in excess of 200 hours have been ob-

tained when the aluminized surface is coated with a uniform silicate layer.

A wide range of sodium silicate solutions can be employed in producing the non-metallic overcoat. For example, the solutions can be prepared from solutions of 50 to 100 percent concentrations of  $\text{Na}_2\text{O} \cdot 3.22 \text{ SiO}_2$ . Various other sodium silicates can be employed to prepare solutions such as Baume 40, 45, 47 and 50. Potassium silicate may be similarly employed. Lithium silicate and also organic silicates can be used, such as ethyl silicate.

A preferred solution for producing a uniform pre-coat or barrier layer on the intermetallic iron aluminide substrate is one containing by weight about 0.05 to 2%  $\text{SiO}_2$  equivalent, for example, a soluble silicate in the form of  $\text{Na}_2\text{O} \cdot 3.22 \text{ SiO}_2$ . The temperature of the substrate during application should preferably range from about 70°C to 95°C.

A preferred method for applying the silicate solution pre-coat at the foregoing concentration comprises immersing the thermally aluminized ferrous component in a tank maintained at a temperature of about 70°C to 95°C with sufficient time in the bath to bring the component to temperature and assure absorption of the solution into the aluminized surface. The excess liquid is then blown off with air and the part allowed to dry. It is immersed again for a brief period for a time sufficient to allow the article to be covered with liquid, after which it is removed, blown off with air and air dried. The steps may be repeated until the desired thickness is obtained. It has been found that when using the air-drying technique, only short dips in the tank need be employed to ensure a continuous build-up of the silicate layer. Leaving the part in the bath too long can result in the layer being redissolved in the solution. To assure wettability of the coating on the intermetallic substrate, an anionic surfactant or wetting agent may be employed, for example, an anionic phosphate surfactant, such as Triton QS-30 (manufactured by Rohm & Haas).

An alternate method which yields a more stable silicate coating resides in applying a succession of layers as described hereinabove followed by curing in an oven. Infra-red or forced air heated ovens may be employed in the temperature range of about 150°C to 430°C (about 300°F to 805°F) with enhanced corrosion protection. The silicate coating applied by any of the methods described herein will produce a uniform layer with a thickness of approximately 0.0001 inch (0.1 mil) while avoiding as far as is possible areas of excess silicate on the surface. A preferred method is to apply at least one pre-coat from a dilute silicate bath containing 0.05 to 2 percent by weight of  $\text{SiO}_2$  equivalent by a series of dipping, drying and curing steps followed by at least one spray coating of silicate from a more concentrated solution containing about 2.5 to 17.5 percent (e.g. 6.8%) by weight of  $\text{SiO}_2$  equivalent.

The advantage of curing the silicate coating which allows multiple layers to be formed is that the cured coating can withstand ten oxidation-corrosion cycles comprising heating the coated substrate to 1000°F (about 538°C) for 1 hour followed by 5 hours of salt spray testing, the foregoing test being repeated for ten cycles. Applications of the silicate coating followed by curing at about 400°F (205°C) have yielded high degrees of protection and, in many cases, very little sacrificial products have been observed after 10 cycles of

heating to 1000°F (538°C) followed by the salt spray test. The foregoing tests are helpful as controls in assuring the quality of the silicate coating before the next coating treatment is applied.

The corrosion resistance of the intermetallic layer is further enhanced by applying a conversion coating to the cured silicate layer. The conversion coating in turn may be covered by a silicate layer. The conversion coating may be applied by spraying, using commercially available reciprocating guns. Following the application of the conversion coating, the silicate solution containing 6.8 percent by weight equivalent of  $\text{SiO}_2$  and containing about 0.002 percent by weight of an anionic phosphate surfactant may optionally be sprayed over the conversion coating having a surface temperature not exceeding about 150°F (65°C) followed by curing at temperatures from about 300°F (150°C) to about 805°F (430°C) for 10 minutes in an infra-red furnace. Another method of covering the conversion coating is to dip the article in a hot solution of about 180°F to 200°F (82°C to 93°C), using a sodium silicate concentration of about 0.9 to 2.4 percent by weight of  $\text{SiO}_2$  equivalent with a 0.002 percent addition of an anionic phosphate surfactant.

The article or component is immersed in the bath and allowed to come to temperature and excess liquid removed rapidly by means of an air gun. It is then immersed again and immediately pulled out of the solution and air dried. A third application is made in the same manner. It is important that excess liquid be removed from the part to avoid foaming during curing. The purpose of repeated immersion and drying is to assure uniform coating of the surface. As stated above, the curing is preferably carried out at about 800°F in an infra-red furnace.

A simple production procedure which has been found successful for applying uniform layers of silicate is as follows:

A component of AMS 5616 steel is subjected to 4 cycles of treatment in the solution by supporting the component, e.g. a vane/shroud component, on a rack which is immersed in the solution and immediately withdrawn. The liquid is allowed to drain for approximately 15 seconds, after which it is immersed again and withdrawn. Following the second dip, air pressure means is disposed about the rack to blow off the excess liquid. This group of steps constitutes one cycle. Four cycles are employed to produce the desired silicate layer. If necessary, an air gun can be used to remove excess liquid from the root of the blades. After the fourth cycle, the blades are dried free of moisture by, for example, blowing with air. The temperature at which the silicate layers are applied may range from about 160°F (70°C) to 200°F (90°C). Following completion of the four cycles, the coating on the dried blade is then cured at about 800°F (425°C) in an infra-red oven.

Apparently the combination of the silicate coating and the aluminide compound in the aluminized surface markedly improves the resistance of the aluminized surface to corrode sacrificially, wherein the life of the sacrificial coating is unexpectedly extended for longer periods of time in saline environments than obtained with the aluminized surface alone.

However, as stated in co-pending application Ser. No. 143,842, the life of the silicated sacrificial aluminized coating is further enhanced by the application of a conversion coating from a solution in substantially

the manner in which the silicate coating is applied. An aqueous conversion coating solution which is preferred may range by weight from about 5 to 30 percent phosphoric acid (preferably 10 to 30 percent), about 0.0235 percent to 3 percent aluminum, about 3 to 8 percent chromic acid ( $\text{CrO}_3$ ), about 0.75 to 6 percent magnesium, and the balance essentially water. A formulation found particularly preferred in producing the solution is as follows:

|                                                                                                                                | Wt. %  |
|--------------------------------------------------------------------------------------------------------------------------------|--------|
| Phosphoric acid                                                                                                                | 15.0   |
| Aluminum powder                                                                                                                | 0.225  |
| Chromic acid ( $\text{CrO}_3$ )                                                                                                | 5.0    |
| Magnesium turnings                                                                                                             | 1.5    |
| A non-anionic surfactant comprising a condensation product of ethylene oxide with an alkylphenol (Triton X-100 by Rohm & Haas) | 0.1    |
| Water                                                                                                                          | 78.175 |
|                                                                                                                                | 100.00 |

The aluminum and magnesium are dissolved in the solution by virtue of the free acid present.

In conversion coating a silicated steel substrate, the substrate is sprayed and then dried and cured in the oven which heats the substrate to a temperature of about 800°F (427°C). The substrate is then cooled prior to the next application of the coating. The steps of spraying, baking and cooling constitute one spray cycle. Three spray cycles are normally used in applying the conversion coating.

The application of the conversion coating as described above results in a smooth uniform surface layer which provides oxidation-corrosion protection without the need for supplementary surface finishing. A buildup of approximately 0.1 mil can be obtained by employing a plurality of silicate and conversion coating application.

It is believed that the baking of the duplex silicate-conversion coating results in a reaction product which provides new and improved resistance to corrosion in saline environments. While the silicate is preferably first applied to the thermally aluminized surface, it is appreciated that it can be applied as a solution together with the conversion coating materials. Thus, the conversion coating solution prior to spraying may contain about 0.05 to 2 percent by weight  $\text{SiO}_2$  equivalent as sodium silicate, potassium silicate, ethyl silicate, and the like.

It will be noted from copending application Ser. No. 143,842 that, in addition to the conversion coating formulation described herein, various conversion coatings of the phosphate-chromate types may be employed in conjunction with the soluble silicate salt. Stating it broadly, the conversion coating comprises phosphates and chromates of at least one metal, for example, Al, Mg, Zn, Be, Ba, Sr, Ce, group metals and other metals. As a preferred embodiment, a conversion coat containing phosphates and chromates of aluminum and magnesium is particularly desirable.

Broadly speaking, the conversion solutions may range in composition by weight of at least about 0.5 percent of at least one phosphate and chromate-forming metal, e.g. about 0.5 to 10 percent, about 5 to 30 percent phosphoric acid, about 3 to 8 percent chromic acid ( $\text{CrO}_3$ ) and the balance essentially water. A preferred conversion solution is one containing by

weight about 0.02 to 3 percent dissolved aluminum, about 0.75 to 6 percent dissolved magnesium, about 5 to 30 phosphoric acid (preferably 15 to 30 percent, about 3 to 8 percent chromic acid and the balance essentially water. A more specific composition is one containing by weight about  $\frac{1}{4}$  percent aluminum, about 1.5 percent magnesium, about 15 percent phosphoric acid, about 5 percent chromic acid and the balance essentially water.

10 Although the present invention has been described in conjunction with preferred embodiments, it is to be understood that modifications and variations may be resorted to without departing from the spirit and scope of the invention as those skilled in the art will readily understand. Such modifications and variations are considered to be within the purview and scope of the invention and the appended claims.

What is claimed is:

1. A method of aluminizing a brazed stainless steel article characterized by at least one brazed joint, the braze of said joint being formed of a non-ferrous brazing alloy of melting point ranging from about 1125°F to 1925°F which comprises:

25 selectively coating the non-ferrous braze of said stainless steel article with an adherent layer of nickel of at least about 0.0002 inch thick, and thermally diffusing aluminum into the entire surface of said article including the selectively coated braze,

30 whereby a sacrificial coating comprising said aluminum is produced, the aluminum coating on the stainless steel surface being characterized by the presence of iron aluminide and the aluminum coating on said nickel-coated braze being characterized by the presence of nickel aluminide.

35 2. The method of claim 1, wherein said nonferrous brazing alloy is either a copper-base, silver-base or gold-base alloy, and wherein said brazing alloy has a melting point ranging from about 1175°F to 1850°F.

40 3. The method of claim 1, wherein said non-ferrous braze alloy on said stainless steel article is selectively coated with nickel by passivating the stainless steel surface of said article and then selectively plating said braze with nickel by immersing said article in a nickel chemical plating bath.

45 4. The method of claim 1, wherein following the production of the thermally diffused aluminum surface, a non-metallic coating is formed on said surface comprising the steps of applying a coating of a solution of a soluble silicate salt selected from the group consisting of sodium silicate, potassium silicate, lithium silicate and ethyl silicate at a temperature ranging up to about 100°C, removing excess liquid from said surface so as to form a uniform layer of said silicate salt covering said surface and then drying and curing said nonmetallic layer, said curing being carried out at a temperature of about 150°C to 430°C.

50 5. The method of claim 4, wherein the step of applying said silicate layer is repeated a plurality of times and dried, and wherein the layers are thereafter cured by heating at a temperature of about 150°C to 430°C.

55 6. The method of claim 4, wherein following the formation of the silicate coating on the aluminum surface, a conversion coating is applied comprising the steps of applying a solution containing by weight about 5 to 30 percent phosphoric acid, about 3 to 8 percent chromic acid ( $\text{CrO}_3$ ), and at least about 0.5 percent of at least

one chromate and phosphate-forming metal and the balance essentially water, drying said conversion coating and then thermally curing said conversion coating.

7. The method of claim 6, wherein said chromate and phosphate-forming metals are aluminum in the amount of about 0.02 to 3 percent, and magnesium in the amount of about 0.75 to 6 percent.

8. A method of aluminizing a brazed stainless steel article characterized by at least one brazed joint, the braze of said joint being formed of a non-ferrous brazing alloy of melting point ranging from about 1125°F to 1925°F and containing by weight at least about 40 percent of at least one metal of the group consisting of copper, silver and gold, and the balance at least one other nonferrous metal which comprises:

selectively coating the braze of said stainless steel article with an adherent layer of nickel by immersing said stainless steel article in a solution containing about 10 to 70 gpl cupric chloride, about 20 to 140 gpl mercuric bichloride, about 10 to 70 gpl bismuth chloride, 100 to 400 ml/l of ethyl alcohol, 100 to 400 ml/l of concentrated hydrochloric acid and the balance essentially water for a time sufficient to effect deposition of mercury at the braze,

dipping said treated stainless steel article into a passivating solution selected from the group consisting of nitric acid, chromic acid and mixtures thereof for a time sufficient to remove the deposited mercury from the braze and thereby activating said braze, subjecting said article to electroless plating by immersing it in a bath of about 15 to 30 gpl nickel sulfate, about 10 to 30 gpl sodium hypophosphite, 20 to 40 gpl sodium glycolate, and 10 to 20 gpl sodium succinate for a time sufficient to produce a nickel deposit on the braze of at least about 0.0002 inch thick,

and then thermally diffusing aluminum into the entire surface of said article including the selectively coated braze,

whereby a sacrificial coating comprising said aluminum is produced, the aluminum coating on the stainless steel surface being characterized by the presence of iron aluminide and the aluminum coating on said nickel coated braze being characterized by the presence of nickel aluminide.

9. The method of claim 8, wherein said nonferrous brazing alloy is either a copper-base, silver-base or gold-base alloy, and wherein said brazing alloy has a melting point ranging from about 1175°F to 1850°F.

10. The method of claim 8, wherein following the production of the thermally diffused aluminum surface, a non-metallic coating is formed on said surface comprising the steps of applying a coating of a solution of a soluble silicate salt selected from the group consisting

of sodium silicate, potassium silicate, lithium silicate and ethyl silicate at a temperature ranging up to about 100°C, removing excess liquid from said surface so as to form a uniform layer of said silicate salt covering said surface and then drying and curing said non-metallic layer, said curing being carried out at a temperature of about 150°C to 430°C.

11. The method of claim 10, wherein the step of applying said silicate layer is repeated a plurality of times 10 and dried, and wherein the layers are thereafter cured by heating at a temperature of about 150°C to 430°C.

12. The method of claim 10, wherein following the formation of the silicate coating on the aluminum surface, a conversion coating is applied comprising the 15 steps of applying a solution containing by weight about 5 to 30 percent phosphoric acid, about 3 to 8 percent chromic acid ( $\text{CrO}_3$ ), and at least about 0.5 percent of at least one chromate and phosphate-forming metal and the balance essentially water, drying said conversion coating and then thermally curing said conversion coating.

13. The method of claim 12, wherein said chromate and phosphate-forming metals are aluminum in the amount of about 0.02 to 3 percent, and magnesium in 25 the amount of about 0.75 to 6 percent.

14. A method of selectively nickel-plating a brazed joint of a stainless steel article wherein the brazed joint is formed from a non-ferrous alloy having a melting point ranging from about 1125°F to 1925°F which comprises: immersing said stainless steel article in a solution containing about 10 to 70 gpl cupric chloride, about 20 to 140 gpl mercuric bichloride, about 10 to 70 gpl bismuth chloride, 100 to 400 ml/l of ethyl alcohol, 100 to 400 ml/l of concentrated hydrochloric acid 30 and the balance essentially water for a time sufficient to effect deposition of mercury at the braze,

dipping said treated stainless steel article into a passivating solution selected from the group consisting of nitric acid, chromic acid and mixtures thereof for a time sufficient to remove the deposited mercury from the braze and thereby activating said braze, and

subjecting said article to electroless plating by immersing it in a bath of about 15 to 30 gpl nickel sulfate, about 10 to 30 gpl sodium hypophosphite, 20 to 40 gpl sodium glycolate, and 10 to 20 gpl sodium succinate for a time sufficient to produce a nickel deposit on the braze of at least about 0.0002 inch thick.

15. The method of claim 14, wherein the nonferrous braze alloy is selected from the group consisting of copper-base, silver-base and gold-base alloys having a melting point ranging from about 1175°F to 1850°F.

\* \* \* \* \*